

June 24, 1930.

E. VON MALTITZ ET AL.

**1,765,955**

## APPARATUS FOR ANNEALING ROLLED METAL PRODUCTS

Filed Jan. 5, 1927



Witness  
Hilton Lenoir

1 Inventors  
Edmund von Maltitz,  
Frederick Wille,  
John F. Jackson,  
Attorney

## UNITED STATES PATENT OFFICE

EDMUND VON MALTITZ, OF GARY, INDIANA, AND FREDRIK WILLE, OF WILMETTE, ILLINOIS, ASSIGNORS TO H. A. BRASSET & COMPANY, OF CHICAGO, ILLINOIS, A CORPORATION OF ILLINOIS

## APPARATUS FOR ANNEALING ROLLED-METAL PRODUCTS

Application filed January 5, 1927. Serial No. 159,072.

This invention relates to a new method of annealing rolled metal products, such as sheets, strips, or wire, made of steel, copper or other metals which can be rolled or drawn.

In the manufacture of such materials it is generally necessary to anneal the rolled or drawn products in order to obtain a perfect product, free from rolling stresses and of a high ductility. The usual way of carrying on the annealing process is to employ so-called annealing boxes wherein the wire or the strip are enclosed during the annealing operation. In order to place this material into these boxes, it is necessary to coil them or cut them into small lengths. The boxes are generally constructed of two separate parts, a bottom and a top, made of heavy cast steel, or of welded or riveted plates. The tops are set on the bottoms and sealed in sand. The seal is necessarily shallow, which often results in air being sucked into the interior of the box during the slow cooling process. These boxes are put into heating furnaces where they are brought up to the proper temperature of annealing. They are generally held in these furnaces for a period of from twelve to twenty-four hours, and are then removed from the furnaces and set to one side for cooling. The control of the temperature is more or less uncertain during this operation, owing to the large number of small units which have to be individually handled and which it is impossible to subject to exactly the same conditions. The process also has the objection of requiring a great deal of labor and of space. The process is also wasteful of fuel, due to the necessity of heating and cooling the great inert mass of the annealing boxes. The equipment for box annealing is large, cumbersome and expensive. The annealing boxes have only a comparatively short life and they are expensive to replace. The loading of the boxes, their charging into the furnace, their heating, drawing and unloading, requires a long time and much labor. For even a moderate tonnage of box annealed wire or strip, the annealing equipment is very extensive.

Furthermore, whereas the annealing process should be carried on in an absolutely re-

ducing or neutral atmosphere so as to avoid oxidation, the drawing in of air causes oxidation of the annealed materials. In the case of cold rolled or cold drawn materials this is particularly objectionable, as a product free from surface oxidation is desired. In the present method of using annealing boxes this cannot be prevented as in the heating of the box and of the charge therein the air entrapped under the cover expands and escapes through the sand seal, whereas when box and charge cool off, a partial vacuum is created and air is drawn in. While the original air contained in the box is not so detrimental to the surface of the metal, as the iron oxide which is formed is reduced again at the high annealing temperatures by the carbon contained in the metal, however, at the lower temperatures which are reached during the latter or cooling period of the annealing process, the temperature is not sufficient for the reaction between the air and the carbon, the affinity of the oxygen for the iron being much greater at the lower temperatures than it is for carbon; consequently, oxidation or scaling of the metal which takes place remains as a defect on the material. This oxidation of the metal in the case of strip steel or wire not only scales the surface but also discolors it and changes a bright surface to one ranging from light straw to light blue in color. While it is possible to prevent air from entering the annealing box during the cooling process by introducing generous quantities of reducing gases under the cover, this is an expensive process, difficult to execute.

Furthermore, for maximum grain refinement, high annealing temperatures are required, and precautions against the material packed in the boxes welding together are expensive. In fact, with box annealing a higher temperature is liable to give just the opposite effect to that obtained with open annealing, viz. the grains in the annealed steel become large, its ductility is correspondingly less, and its brittleness is greater, for the reason that the cooling of the steel in the boxes is very slow, which gives ferrite the opportunity to form in large crystals, resulting in a brittle steel of low ductility, while in our

method of annealing hereinafter described, the cooling down from the critical temperature is fast and no opportunity is given to form large grains of ferrite. Another drawback of box annealing is the uneven temperature between the outer and inner portions in the case of annealing coils of wire or of strip, which with very careful work may be reduced to a difference of about 50 degrees 10 Fahr., but which is still too great to produce a uniform material well annealed throughout.

We have invented a new method which prevents oxidation of the steel or other metals 15 during the annealing process, which provides better control of the temperature during the annealing process and a more uniform application thereof to the metal, and which greatly reduces the labor and fuel cost of the 20 annealing process and requires much less space in its operation.

Our invention will be better understood by referring to the attached drawing showing a preferred method of applying our invention. On the drawing is shown a vertical cross-section of a continuous annealing furnace, in which 1 is a piece of strip steel or rolled or drawn wire fed in over the roller 2, into a seal box or chamber 3. The material 25 is carried around a roller 4, and up through a vertical riser chamber 5, which preferably is equipped with radiating ribs 6 on its inner surface. The seal chamber 3 and the vertical riser chamber 5 are filled with a sealing material, such as charcoal or sand, or a mixture 30 of both, or other material which will prevent the access of air. This material fulfills the purposes of pre-heating the metal, and the charcoal at the same time acts as a reducing agent in respect to the air which 35 might be carried into the apparatus with the steel. The sealing chamber 3 is heated by a combustion chamber 7 with gas, oil or other convenient fuel, the waste gases of 40 which pass upward and around the riser chamber 5 through jacketed space 8 and out through stack 8<sup>a</sup>, the heat from the waste gases being transmitted through the walls of the same and through the radiating fins 45 into the sealing material which surrounds 50 the sheet, strip or wire which is to be annealed.

From chamber 5 the strip or wire passes through an annealing furnace comprising a 55 communicating series of vertical annealing chambers, as 10, 10<sup>a</sup>, 10<sup>b</sup>, 10<sup>c</sup> and 10<sup>d</sup>, being guided through the same over rollers 9, 9<sup>a</sup>, 9<sup>b</sup>, 9<sup>c</sup>, 9<sup>d</sup> and 9<sup>e</sup>. These chambers are preferably heated electrically by heating elements, 60 as 11, 11<sup>a</sup>, 11<sup>b</sup>, 11<sup>c</sup>, 11<sup>d</sup>, 11<sup>e</sup>, 11<sup>f</sup>, 11<sup>g</sup>, 11<sup>h</sup>, but they can also be heated by other means, the heat being preferably radiated from vertical partition walls when other than electric heaters are used; in the case of electric heaters 65 these in themselves form the partitions. At

the bottom of these annealing chambers provision is made for a charcoal bed 3<sup>a</sup>, which may be heated from below by another combustion chamber 7<sup>a</sup>, or by additional electric current. The top of the annealing chambers is sealed by covers 12, 12<sup>a</sup>, 12<sup>b</sup>, which are sealed air tight and can be readily removed for quick inspection or exchange of rollers and heating elements. At the end of the annealing chambers, preferably at the 70 bottom of the last one, is another seal box 13 filled with sand or other sealing material, through which the strip of metal, or strand of wire, is carried over roller 14 into a cooler 15, which may be a sectional pipe or box, 75 preferably made of copper or other metal of high heat conductivity, having radiating ribs 16 on its outside surface, to facilitate quick cooling. Rollers 17, 17<sup>a</sup> located at the top and bottom of this box carry the material down through a similar section 15<sup>a</sup> of the cooler into seal box 18 filled with oil or water, or other sealing liquid or solid, as may be required to give the best finish to the material. We have found that oil at a moderate 80 temperature is particularly effective in preventing oxidation of annealed material.

While the apparatus as described presents the simplest form to carry out our invention, many variations may be used. For instance 85 another method is to carry the strip or wire parallel to the electric heater elements or heated partition walls, and centrally between them, by feeding it over pairs of rollers instead of singles at the top and bottom of the 90 chambers.

To start the operation, the strip or wire is fed over the rollers in the furnace, which can readily be done by hand, the lids 12 being removed and the sealing boxes being empty. 105 When the first piece, which may or may not be of the same kind that is to be annealed, has been pulled through so that its ends protrude from opposite ends of the furnace, the strip or wire to be annealed is welded on to it 110 by spot welding at the feed side of the furnace. It can also be fastened on by other means, and in case of wire it can be hooked onto the perforated feeder strip. The seal boxes are then filled, the heat is turned on, 115 and the strip or wire is slowly moving through the annealing furnace by any suitable power operated means capable of speed regulation, at a rate of speed which can be accurately calculated to carry through the annealing process exactly to the theoretical requirement. The temperature is carefully controlled by pyrometers inserted at various points of the annealing chambers. If the pyrometers indicate too high or too low a 120 temperature, the speed is increased or decreased, which effects an immediate change, the result being much quicker than that of increasing or decreasing the heat, which can be done as a secondary remedy. When al- 125 130

most the entire length of a strip of wire or coil to be annealed has been fed into the furnace, the next piece is welded or fastened onto the end of the first one, and so on, so that the 5 annealing operation may go on continuously from the time it has been first started without any interruption of the process. Changes can be made from wide strips to narrow strips without stoppage of the operation, or even 10 from heavy wire to light wire, and as a matter of fact from one material to another, if such an occasion should arise, providing only that the same can be welded or fastened together mechanically.

15 It will be readily seen that this method of annealing guarantees the presence at all times of a neutral or reducing atmosphere. At the very start of the operation, the original air contained in the chamber is quickly expanded 20 by heating, and displaced by the evolution of carbon monoxide gases from the charcoal contained in the seal box and the annealing chamber; during the process this is augmented by the carbon monoxide and hydrogen gas evolved from the annealing steel, 25 whereby a slight pressure is automatically maintained in the annealing chambers, preventing any possible drawing in of air.

30 The highest desirable annealing temperatures can be carried without the danger of welding closely packed material together as in box annealing, and the rapid cooling prevents the formation of large grains of ferrite, thus giving a metal of highest possible 35 ductility.

Another advantage of this method of annealing is that it is carried on with the material in a vertical position suspended freely and not in contact with any surface except 40 that of the rollers, which are driven and therefore present no friction surface. Thereby damage to the surface of the material is prevented. The material in the seal box is fine sand and charcoal, the charcoal being soft, 45 and the fine sand having an effect of polishing the material. There is no opportunity anywhere in this operation for the material to become scratched, which is one of the important features of this invention, much of 50 the good material being destroyed in the box annealing process through scratches.

While we have described a method particularly adapted for annealing and heat treating strip steel and wire, it will be understood 55 that the same process can be carried out by a different design of apparatus, by employing various heating means, and other means of sealing, transporting and cooling the material without deviating from this invention. 60 Also while this process has been particularly developed to treat steel products, it is equally applicable to other metals which require annealing or heat treating.

It should be understood that the term 65 "strip" is used in the claims in a generic sense,

to comprehend any elongated flexible form in which the material to be treated may be fashioned, whether it be in the form of a thin flat band, such as is ordinarily termed a strip, or in the form of wire, or of links connected in the form of a chain, &c. 70

In addition to the aforesaid process our invention includes also the apparatus illustrated and described.

What we claim as our invention and desire 75 to secure by Letters Patent, is—

1. In a device of the class described, the combination of a heating furnace and an annealing chamber comprising a continuous zigzag passageway in which the passes are disposed substantially vertically, the passes in the furnace being separated by walls adapted to give off heat to the material between them, and the passes in the annealing chamber being separated by walls adapted to 80 dissipate heat, a U-shaped seal between the furnace and the annealing chamber filled with granular material and having a circular guide over which the strip to be treated is trained, an entrance seal of granular material for the furnace, and a liquid seal for the exit of the strip from the annealing chamber. 85

2. In a device of the class described, the combination of a heating chamber comprising a zigzag passageway consisting of substantially vertical passes, and an annealing chamber comprising substantially vertical passes, heat supplying walls for the vertical passes in the furnace, and heat dissipating walls for the passes in the annealing chamber, and a granular U-shaped seal separating the passes of the furnace from the passes of 90 the annealing chamber. 95

3. In a furnace of the class described, a heating chamber comprising side and end walls, granular material disposed in the bottom of the chamber, a U-shaped outlet from the chamber filled with granular material, a zigzag passageway comprising substantially vertical passes disposed within the chamber, said passes being separated by heat supplying walls contained within the chamber, removable cover means for the passes of the chamber, means for heating the incoming strip of material comprising a substantially U-shaped passageway filled with granular material and containing a guide in the bottom of the U, and heating means for heating 105 said granular material. 110

4. In a device of the class described, a zigzag passageway comprising a plurality of passes, means for training a continuous strip through the passageway, means for sealing off one part of the passageway from the remainder, means for heating the passes in said one part, and means for cooling the passes of the remainder, and a liquid outlet seal for the last pass. 120

5. In a device of the class described, a cool- 130

ing chamber comprising a plurality of substantially vertical passes, each pass being defined by a tubular heat radiating wall, and a roller at the junction of each pair of passes for conducting a metal strand through said passes out of contact with the wall thereof.

6. An annealing chamber comprising an inverted U-shaped passageway having a roller at the upper end of the passageway for 10 guiding a strip to be annealed, the walls of the passageway being defined by metallic heat radiating members, a U-shaped granular inlet seal for the introduction of a heated metallic strip, and a U-shaped liquid outlet seal 15 for withdrawing the strip from the annealing chamber.

7. In a device of the class described, the combination of a closed heating chamber comprising a generally zig-zag passageway 20 consisting of substantially vertical passes, heat supplying walls forming parts of the passes, rollers at the junctions of the passes for forwarding a metal strand to be treated out of contact with the walls of the passes 25 and an annealing chamber comprising substantially vertical passes, said latter chamber comprising heat dissipating walls and having strand forwarding rollers for forwarding the metal strand out of contact with the walls, 30 and a granular U-shaped seal separating the passes of the furnace from the passes of the annealing chamber, there being removable portions at the upper end of the heating chamber and at the upper end of the annealing chamber to facilitate training of the metal strand over the rollers.

8. In combination, an annealing chamber having an entrance chamber provided with a seal of charcoal and providing a zig-zag passageway having an outlet seal of granular material, means for passing a metal strip through said entrance seal, said passageway and outlet seal and maintaining the strip out of contact with the walls of said chamber, 45 and means for heating said entrance chamber for bringing the strip to an annealing temperature.

9. In combination, an annealing chamber having an entrance chamber provided with a seal of charcoal and providing a zig-zag passageway having an outlet seal, a cooling chamber having walls for dissipating heat, an exit seal for the cooling chamber, means for passing a metal strip through said entrance seal, said passageway, said outlet seal and cooling chamber, while maintaining the strip out of contact with the walls of said chambers, and means for heating said entrance chamber to bring the strip to an annealing temperature.

EDMUND von MALTITZ.  
FREDRIK WILLE.